

## UNITED STATES PATENT OFFICE

2,658,870

## CUTTING OIL COMPOSITION

Henry A. Ambrose, Penn Township, Allegheny County, and Oliver L. Brandes, Gibsonia, Pa., assignors to Gulf Research & Development Company, Pittsburgh, Pa., a corporation of Delaware

No Drawing. Application March 3, 1952,  
Serial No. 274,678

3 Claims. (Cl. 252—48.6)

1

This invention relates to a cutting oil composition and more particularly to an oil adapted to be applied as a thin high-speed jet into the angle between the work and the cutting edge of a metal-working tool.

The use of cutting oils to carry off excess heat and to lessen friction created during metal-working operations such as turning, boring, milling, and shaping, is recognized as necessary to the successful commercial operation of such processes. Improved techniques in applying a cutting fluid to the surface of the metal being worked have presented problems which heretofore have not been encountered.

The application of a cutting oil to a surface being worked has generally comprised flowing over the tool either by gravity or under low pressure, a large amount of a cutting oil, the theory being that by flooding the working surface with a cutting oil the heat would be dissipated, the metal chips washed away, and the cutting operation lubricated by the quantity of the oil used.

Recent developments have shown that the application of a cutting oil in the form of a thin high-speed jet to the angle between the work and the tool increases the life of the tool while, at the same time, the surface of the finished work is improved. When the cutting oil is applied as a thin high-speed jet, the oil penetrates the extremely small clearance between the work and relief surface of the tool without impinging upon the heel of the tool or otherwise dissipating its energy before reaching its destination. The prior cutting oil compositions which have been employed when the flooding technique is used are not entirely satisfactory when applied as a high-speed jet.

We have discovered that an improved cutting oil composition adapted to be applied as a thin high-speed jet is obtained by incorporating in a major amount of a mineral lubricating oil having a viscosity of about 70 to about 300 SUS at 100° F. a minor amount of (1) a mineral lubricating oil having a viscosity between about 100 and about 200 SUS at 210° F., (2) a fixed fatty oil, and (3) the residue which remains after removal of the solvent from the extract obtained by extracting a petroleum distillate oil with a solvent capable of removing polycyclic hydrocarbons and sulfur compounds from petroleum distillate oils, said residue having a viscosity between about 55 and about 70 SUS at 210° F.

2

We have found that the base oil for the cutting compositions of this invention should be a mineral oil fraction having a viscosity of about 70 to about 300 SUS at 100° F. The lower viscosity oils, i. e., those having a viscosity not greater than about 40 SUS at 100° F., which oils are satisfactory when the flooding technique is used, are not satisfactory when the high-speed jet technique is employed. For instance, we have found that a cutting oil composition having as its base a mineral seal oil having a viscosity of about 35 SUS at 100° F. gave strikingly poorer results than a cutting oil composition having as its base a mineral oil having a viscosity of about 100 SUS at 100° F. A particularly advantageous mineral oil in the compositions of our invention is a light Texas oil, a typical example of which has an API gravity of about 24, a flash point of about 320° F., a fire point of about 355° F., a viscosity of about 100 SUS at 100° F., a color of about 2 on the NPA scale, and a pour point of about -45° F. In the cutting oil compositions of the present invention, the 70 to 300 SUS oils constitute at least 50 per cent by weight of the total composition and advantageously are used in amounts of about 75 to about 98 per cent by weight.

A mineral lubricating oil having a viscosity of about 100 to about 200 SUS at 210° F. is employed in the compositions of our invention to provide a film of lubricant on the metal surface which is more stable to the high temperatures encountered than the mineral oil which forms a base for the cutting oil compositions. A lubricating oil which is particularly advantageous for this purpose is an unfiltered bright stock having a viscosity of about 150 SUS at 210° F. This highly viscous oil component of the cutting oil compositions of our invention is employed in an amount between about 1 and about 20 per cent by weight.

The fixed fatty oils used in the compositions of our invention are employed primarily to increase the oiliness or lubricity of the resultant compositions and are customarily used in amounts between about 0.5 and 15.0 per cent by weight. Examples of the fixed fatty oils which may be used are lard oil, tallow oil, neat's-foot oil, sperm oil, wool oil, whale oil, and the like. Of these oils, lard oil is particularly satisfactory. Instead of the animal oils we may substitute therefor fish oils or vegetable oils. The fish oils are generally less desirable because of their offensive odor. The vegetable oils are less desirable than

the animal oils because of their tendency to oxidize and form gum at the temperatures encountered in cutting operations. By using a sufficient amount of a scenting agent such as pine oil, oil of citronella, and the like, the offensive odor of the fish oils may be overcome. Likewise, by employing a sufficient amount of an oxidation inhibitor such as, for example, an amino phenol, an alkylated phenol, an alkyl phosphite, and an alkylated phenol phosphite or phosphate ester, the oxidation of the vegetable oils such as olive oil, rapeseed oil, corn oil, and castor oil, may be minimized. For this purpose the alkylphenyl phosphite esters, which are also effective extreme pressure agents, are particularly advantageous. Typical compounds within this class are tri-(tertiary-amyl-phenyl)-phosphite and tri-butyl phosphite. When an oxidation inhibitor is employed, an amount between about 0.03 and about 5.0 per cent by weight may be used. The amount of a scenting agent employed will depend upon the oil and the particular agent used, the amount ordinarily not exceeding about 0.1 per cent by weight.

The residue which remains after removal of the solvent from the extract obtained by extracting a petroleum distillate oil with a solvent capable of removing polycyclic hydrocarbons and sulfur compounds from petroleum distillate oils is incorporated in the compositions of the invention to increase further the extreme pressure characteristics of the compositions. Solvent refined extracts obtained from distillate oils and having viscosities of 55 to 70 SUS at 210° F. are most satisfactory. The solvent employed in treating the petroleum distillate oil to obtain the residue may be furfural, nitrobenzene, sulfur dioxide, phenol, and the like. The residue is advantageously used in an amount between about 1 and about 10 per cent by weight based on the weight of the total composition. A typical residual product of this type has the following properties:

|                 |      |
|-----------------|------|
| Gravity, °API   | 14.4 |
| Flash point, °F | 365  |
| Fire point, °F  | 435  |
| Viscosity, SUS: |      |
| At 100° F       | 1222 |
| At 210° F       | 61.8 |
| Pour point, °F  | +5   |

The cutting oil compositions of this invention may contain other "additive" agents, if desired, to improve other specific properties without deleteriously affecting the beneficial properties of the compositions. For example, wetting agents such as fatty acids and detergent sulfonates may be incorporated in the compositions to improve their properties for wetting the metal surfaces with which they come in contact. Also, if desired, the oil may contain foam inhibitors such as organo-silicon oxide condensation products, organo-silicol condensation products, and the like.

The increased tool life obtained when employing compositions of the present invention in a high-speed jet cutting mechanism as compared with a similar composition prepared from an oil having a viscosity below about 70 SUS at 100° F. is illustrated in Table I. The tool life data were obtained when cutting AISI 3140 steel, at a speed of 140 surface feet per minute, and a depth of cut of 0.150 inch.

4  
Table I

| Composition                                                                                                            | A     | B     | C     | D    |
|------------------------------------------------------------------------------------------------------------------------|-------|-------|-------|------|
| Mineral Oil Base, parts by weight                                                                                      | 95    | 85    | 95    | 95   |
| Lard Oil, do                                                                                                           | 2     | 6     | 2     | 2    |
| Refined lubricating oil having a viscosity of 150 SUS at 210° F. and a pour point of +5° F., parts by weight           | 2     | 6     | 2     | 2    |
| Naphthenic furfural extract of coastal distillate, 55 to 70 SUS at 210° F. and a pour point of +5° F., parts by weight | 1     | 3     | 1     | 1    |
| Tool Life, minutes                                                                                                     | 340   | 335   | 325   | 210  |
| Typical properties of the Mineral Oil Base:                                                                            |       |       |       |      |
| Gravity, °API                                                                                                          | 24.1  | 24.1  | 25.8  | 41.0 |
| Viscosity, SUS, at 100° F                                                                                              | 103.5 | 103.5 | 74    | 38   |
| Flash point, °F                                                                                                        | 320   | 320   | 295   | 260  |
| Fire point, °F                                                                                                         | 355   | 355   | 345   | 305  |
| Pour point, °F                                                                                                         | -45   | -45   | below | 25   |
| Color, NPA                                                                                                             | 1.75  | 1.75  | 1.5   | 1-   |

As can be noted from the tool life data, compositions of the invention, compositions A, B, and C, are strikingly superior to a composition not within the scope of the invention, i. e. composition D.

Composition A represents a preferred embodiment of the invention and has an API gravity of 24.5; viscosities of 114 SUS and 39.1 SUS at 100° and 210° F., respectively; NPA color of 3+; a pour point of -57° F.; a flash point of 320° F.; and a fire point of 360° F.

The tool life tests referred to hereinabove were made on AISI 3140 steel using a high-speed steel (18-4-1) tool. In these tests the cutting compositions were directed in the form of a thin jet of cutting liquid at a velocity of about 260 feet per second and delivering 0.12 gallon per minute into the angle between the work and the tool. The thin jet was obtained by passing the cutting composition through a small orifice (0.014 inch) in a nozzle which was mounted on the carriage of the lathe. In the present tests a one-half inch tool bit was employed. The cutting compositions were supplied to the nozzle at a temperature of about 100° F. under a pressure of 400 pounds per square inch. In these tests a conventional overhead stream of cutting composition circulating about 3 gallons per minute was also employed.

While the invention has been described above with reference to certain specific embodiments thereof by way of illustration, it is to be understood that the invention is not limited to such embodiments except as hereinafter defined in the appended claims.

We claim:

1. An improved cutting oil composition adapted to be applied as a thin high-speed jet consisting of at least 50 per cent by weight of a mineral lubricating oil having a viscosity of about 70 to about 300 SUS at 100° F.; about 1 to about 20 per cent by weight of a mineral lubricating oil having a viscosity between about 100 and about 200 SUS at 210° F.; about 0.5 to about 15 per cent by weight of a fixed fatty oil; and about 1 to about 10 per cent by weight of the residue which remains after removal of the solvent from the extract obtained by extracting a petroleum distillate oil with a solvent capable of removing polycyclic hydrocarbons and sulfur compounds from petroleum distillate oils, said residue having a viscosity between about 55 and about 70 SUS at 210° F.

2. An improved cutting oil composition adapted to be applied as a thin high-speed jet consisting of about 75 to about 98 per cent by

weight of a mineral lubricating oil having a viscosity of about 70 to about 300 SUS at 100° F.; about 1 to about 20 per cent by weight of a mineral lubricating oil having a viscosity between about 100 and about 200 SUS at 210° F.; about 0.5 to about 15 per cent by weight of lard oil; and about 1 to about 10 per cent by weight of the residue which remains after removal of the solvent from the extract obtained by extracting a petroleum distillate oil with a solvent capable of removing polycyclic hydrocarbons and sulfur compounds from petroleum distillate oils, said residue having a viscosity between about 55 and about 70 SUS at 210° F.

3. An improved cutting oil composition 15 adapted to be applied as a thin high-speed jet consisting of about 95 per cent by weight of a mineral lubricating oil having a viscosity of about 100 SUS at 100° F.; about 2 per cent by weight of a mineral lubricating oil having a 20 viscosity of about 150 SUS at 210° F.; about 2

per cent by weight of lard oil; and about 1 per cent by weight of the residue which remains after removal of the solvent from the extract obtained by extracting a petroleum distillate oil with a solvent capable of removing polycyclic hydrocarbons and sulfur compounds from petroleum distillate oils, said residue having a viscosity between about 55 and about 70 SUS at 210° F.

HENRY A. AMBROSE.  
OLIVER L. BRANDES.

## References Cited in the file of this patent

## UNITED STATES PATENTS

| Number    | Name      | Date          |
|-----------|-----------|---------------|
| 2,010,606 | Moser     | Aug. 6, 1935  |
| 2,308,427 | Roehner   | Jan. 12, 1943 |
| 2,453,708 | Hughes    | Nov. 16, 1948 |
| 2,470,913 | Bjorksten | May 24, 1949  |